

Dec. 18, 1962

A. J. DEYRUP

3,069,333

CHROMIUM PLATING

Filed July 25, 1961

FIG. 1



FIG. 2



INVENTOR

ALDEN J. DEYRUP

BY *Louis A. Wible*

ATTORNEY

# United States Patent Office

3,069,333

Patented Dec. 18, 1962

1

3,069,333

## CHROMIUM PLATING

Alden J. Deyrup, West Chester, Pa., assignor to E. I. du Pont de Nemours and Company, Wilmington, Del., a corporation of Delaware

Filed July 25, 1961, Ser. No. 126,623  
17 Claims. (Cl. 204—51)

This invention relates to chromium plating, and more particularly it relates to chromium plating from a new and improved electrolytic plating bath.

This application is a continuation-in-part of my co-pending application Serial No. 33,951, filed June 6, 1960, now abandoned, which in turn is a continuation-in-part of application Serial No. 844,875, filed October 7, 1959, now abandoned.

The present commercial chromium plating processes are based on the electrolysis of chromium trioxide,  $\text{CrO}_3$  (chromic acid), solutions containing small amounts of a catalyst, e.g., sulfates, fluorides or the like. In such commercial processes, for the production of bright plates of acceptable quality the current density and temperature during plating must be closely controlled. Even when closely controlling the current density, temperature and chromic acid-catalyst ratio, the throwing power of the plating bath is very low as compared to other metal plating processes. Because of poor throwing power, it is necessary to provide anodes conforming to the shape of the object to be plated. Moreover, the current efficiency of the commercial plating baths are usually no greater than 8-12% and under the most optimum conditions only 15-20%.

Also, objectionably large volumes of oxygen and hydrogen are given off during plating as a result of which a highly noxious and corrosive spray of chromic acid is always present over the plating bath during the plating operation. Again, large amounts of chromic acid are lost by drag-out and spray due to the necessity of employing rather highly concentrated amounts of chromic acid in commercial baths. The art also discloses chromium plating processes employing trivalent chromium salts. Such previously known trivalent chromium plating processes have had no commercial significance.

It is an object of this invention to provide a new and improved electrolytic chromium plating bath.

It is another object to provide electrolytic chromium plating baths that have relatively good throwing power, and improved current efficiency.

It is another object to provide a new and improved electrolytic chromium plating bath in which the chromium is plated from a divalent chromium salt.

It is yet another object to provide a new and improved electrolytic chromium plating process that will exhibit improved current efficiency and throwing power and will produce an acceptable bright chromium plate.

It is a further object of this invention to provide a new and improved electrolytic chromium plating process that will deposit a new and different form of chromium having an exceedingly high tensile strength.

It is yet another object to produce a self-sustaining chromium foil having a high tensile strength.

Other objects of the invention will become apparent by reference to the following description and claims.

The objects of this invention may be accomplished, in general, by preparing an electrolytic aqueous chromium plating bath comprising a chromium salt in which the chromium has the valence of 2 (hereinafter referred to as a divalent chromium salt), at least one carboxylic acid taken from the group consisting of formic and glycolic acids, and an alkali metal salt taken from the group consisting of sodium and potassium formates and glycolates, and sodium and potassium salts of a strong acid, i.e., an

2

acid having a dissociation constant greater than  $10^{-2}$ . The dissociation constant K is defined as

$$K = \frac{(\text{H}^+)(\text{A}^-)}{(\text{HA})}$$

where  $(\text{H}^+)$ ,  $(\text{A}^-)$  and  $(\text{HA})$  are respectively the molar concentrations of hydrogen ion, acid anion and undissociated acid. Many of the strong acids such as  $\text{HCl}$  and  $\text{H}_2\text{SO}_4$  have dissociation constants too large to measure, much greater than  $10^{-2}$ , so they ordinarily do not appear in published tables of dissociation constants. The bath may also advantageously contain boric acid, and, if boric acid is present, it may also advantageously contain sodium fluoride. Boric acid and/or sodium fluoride are not however essential ingredients of the chromium plating bath of this invention.

This electrolytic plating bath may be operated electrolytically at room temperature, or at elevated temperatures up to  $90^\circ \text{C}$ , to deposit bright continuous, highly corrosion-resistant chromium plate. The metallic surface to be plated is first thoroughly cleaned in accordance with cleaning procedures well established in the art. Preferably, the metallic surface to be plated, e.g., a copper or nickel surface, is smooth and polished so as to produce a bright chromium plated finish. The metallic object to be plated is suspended as the cathode in the aforesaid electrolytic bath and spaced fairly evenly from an inert anode, e.g., a carbon or graphite anode. The plating may be carried out by passing an electric current of 30 to 120 amps./sq. ft. at room temperature up to 200-450 amps./sq. ft. at elevated temperatures above  $60^\circ \text{C}$ . between said cathode and anode.

In comparison with the trivalent-chromium plating baths described and claimed in my Patent No. 3,006,823, the present divalent-chromium plating baths have higher current efficiencies, higher maximum plating speeds and produce a whiter chromium deposit.

It has, moreover, been found, in accordance with this invention, that under certain specific conditions as hereinafter set forth, it is possible to produce a new and previously unknown form of chromium having an exceedingly high tensile strength, being completely self-supporting even in the form of a thin electroplated film, having very different electrical resistivity and temperature coefficient of resistivity than previously known chromium and being very useful in the form of films or foils.

Such unique form of chromium may be obtained by the electrolytic deposition from the above-described chromium plating bath when the sole carboxylic acid present is formic acid, the sole carboxylate is sodium or potassium formate, the plating temperature is above  $50^\circ \text{C}$ . and the bath contains less than 10 parts per million of either sulfur or selenium, impurities normally found in chromium.

The accompanying illustrations are drawings of X-ray diffraction patterns of chromium electrodeposits, in which:

FIGURE 1 illustrated the X-ray diffraction pattern of chromium produced by the conventional commercial hexavalent chromium plating process, and

FIGURE 2 illustrates the X-ray diffraction pattern of chromium produced by the divalent chromium plating process of this invention.

Referring to the drawings, the sharp distinction between successive X-ray diffraction bands in FIGURE 1 clearly indicates that the chromium deposited from the prior art hexavalent process has a distinct crystallinity of large well-defined crystals. The wash'd-out indistinct X-ray diffraction bands shown in FIGURE 2 designate a lack of distinct, well-defined crystallinity or crystals of an exceedingly small size.

The plating baths of this invention are greatly superior to commercial hexavalent chromium plating baths in

current efficiency, throwing power and plating range. These terms are, for convenience, defined as follows:

"Current efficiency" is generally defined as the ratio of weight of metal actually deposited by a given current for a given time to that which would have been deposited if electro-reduction of the desired metal were 100% efficient. The latter is calculated from Faraday's law, which says that 96,500 coulombs (ampere-seconds) is required to electrodeposit one gram equivalent of metal, if no side-reactions occur such as liberation of hydrogen. Current efficiency is commonly expressed as percent. It is important to note that current efficiencies as thus calculated are not directly comparable between VI, III, and II-valent chromium. Thus, the best that could possibly be deposited by 96,500 coulombs from hexavalent, trivalent, and divalent chromium salts are, respectively,  $52 \div 6$ ,  $52 \div 3$ , and  $52 \div 2$  grams. Thus, a current efficiency of 15% with a trivalent bath is just as good as 30% with a hexavalent bath, or only as good as 10% with a divalent bath. Current efficiency is important because it governs in part the rate of plating, and so is of great economic importance. However, the cost of current is only one factor in the economics of plating. Probably of more practical importance is the maximum speed of plating, using as much current as will be tolerated without appearance of defects discussed below under "plating range."

"Throwing power" is a term used in the plating industry to signify the degree to which plating occurs in recesses or on surfaces which are remote from the anode as compared with plating on flat surfaces or those near to the anode. Every one in the plating industry knows what "good throwing power" is, and that commercial chromium plating baths have very poor "throwing power." However, there does not appear to be a generally accepted measure of "throwing power" as such. To a principal degree, the differences in plating on the variously disposed surfaces of an article in a plating bath are governed by the response of the plating system to the local current densities. Therefore, we can secure good information about "throwing power" by measuring "plating range."

It is frequently true of electroplating baths that below certain current densities (amperes per unit area) they either do not deposit metal at all, or if they deposit metal, it is defective in brightness, color, or other respect. Above an upper limiting current density characteristic of each specific bath the plating is "burned" or discolored, matt, spongy, or otherwise defective. Between these limits, which I will call "threshold current density" and "ceiling current density," good plating occurs. It is evident that if this "plating range" is very narrow, the system will have "poor throwing power." This is a present handicap in commercial chromium plating. It is also evident that if this range is very broad and the "ceiling current density" occurs at very heavy currents, then plating can be very rapid, even if current efficiency is only moderately good.

The divalent chromium salt may be composed of any chromous compound which will dissolve in the plating bath and which will not introduce into the said bath non-oxidizing anions. For example, chromous chloride,  $\text{CrCl}_2$ ; chromous bromide,  $\text{CrBr}_2$ ; chromous iodide,  $\text{CrI}_2$ ; chromous fluoride,  $\text{CrF}_2$ ; chromous formate,



chromous glycolate,  $\text{Cr}(\text{CH}_2\text{OH}\cdot\text{CO}_2)_2\cdot\text{H}_2\text{O}$ ; or chromous sulfamate,  $\text{Cr}(\text{SO}_3\text{NH}_2)_2$ , may be used for this purpose.

The chromous salts of acids having an ionization constant greater than  $10^{-2}$  are preferred, however, a few chromous salts of acids having an ionization constant less than  $10^{-7}$  such as chromous carbonate may also be used. Except for chromous formate and/or chromous glycolate, chromous salts of acids having ionization constants between  $10^{-2}$  and  $10^{-7}$  are much less desirable because of low plating efficiency. When it is desired

to use a bath containing a fluoride, it has been found most expedient to use sodium fluochromate (II),  $\text{Na}_2\text{CrF}_4$ ; or when it is desired to use a bath containing boron but not containing the fluoride, it is advantageous to use a compound,  $\text{CrOHX}\cdot\text{H}_3\text{BO}_3$  (X=Cl, Br, or I). These compounds are air-stable salts, whereas many chromous salts are not air stable and, therefore, must be protected from the atmosphere during shipping and handling.

10 The preparation of  $\text{Na}_2\text{CrF}_4$  is described and claimed in my U.S. Patent No. 2,996,353. The preparation of compounds of the formula  $\text{CrOHX}\cdot\text{H}_3\text{BO}_3$  is described in my copending application, Serial No. 118,788, filed June 22, 1961.

15 The carboxylic acid present in the plating bath must be formic acid or glycolic acid or a mixture thereof. It may be added either as the acid itself or as an alkali metal formate or glycolate together with a strong acid such as hydrochloric acid (an acid having a dissociation constant of at least  $10^{-2}$ ) which will react to produce the desired formic or glycolic acid in situ, care being taken to avoid an excess of the strong acid which might reduce the pH below about 1.7.

In general, an alkali metal formate, glycolate, or mixture thereof may be present as the sodium or potassium salt of either of these acids. The alkali metal carboxylate need not be derived from the same carboxylic acid as the carboxylic acid used in making the bath. For example, the carboxylic acid may be formic acid, and the alkali 20 metal carboxylate may be added as sodium glycolate. It is not necessary in all cases to have an alkali metal formate or glycolate present in the bath, although sometimes it is preferable. If the bath contains no alkali metal carboxylate, then it is essential to have present in the 25 bath an alkali salt of a strong acid (dissociation constant  $>10^{-2}$ ), as, for example, sodium chloride.

In cases where fluoride is used in the bath, it should be sodium fluoride. In the absence of fluoride, alkali salts may be present, and are usually desirable to improve conductivity, and these may be either sodium or potassium or, in some cases, ammonium salts. However, when fluorides are used in the bath, potassium and ammonium salts from any source are undesirable because they may remove both fluorine and boron as insoluble fluoborates.

30 40 45 50 55 The divalent chromium salt, when used, may be added as borax, boron oxide, boric acid, or sodium oxyfluoborate, a complex compound having the formula  $4\text{NaF}\cdot 5\text{B}_2\text{O}_3$  (see U.S. Patent No. 2,823,095). All of these materials are equivalent to boric acid in aqueous solution and react to form the desired  $\text{BF}_3\text{OH}^-$  ion further discussed below. Although fluoborates, i.e., the well-known compounds containing the  $\text{BF}_4^-$  ion, may be used as the source of boron, they are not recommended since the baths are not satisfactory for a period of days until the fluoborates have had time to hydrolyze to make the desired complexes.

The essential components of the plating bath are (1) a divalent chromium salt, (2) formic acid or glycolic acid or mixtures thereof, and (3) either an alkali formate or glycolate or mixture thereof, or an alkali salt of a 60 strong acid (dissociation constant  $>10^{-2}$ ). In addition to these essential components, desirable components for some purposes are boric acid or boron acid and sodium fluoride. The above-described essential and nonessential but desirable components of the plating bath may be 65 constituted of compounds which may comprise one or more of these components. For example, sodium oxyfluoborate may be the source of both the fluoride and the boric acid; or the sodium fluochromate may be the source of both the essential divalent chromium salt and the fluoride; or chromium formate may be the source of both the divalent chromium and the formate radical. The essential constituents of the electroplating bath of this invention are preferentially present in the plating bath in certain proportions. This is also true of the desirable 70 but nonessential constituents. In 1000 grams of plating

solution, it is preferred that the several constituents be present in about the following number of gram moles depending, of course, upon the particular compounds used, it being understood that the constituents may be present in complex chemical combinations and reference to amounts of the following specific compounds is to be regarded from the standpoint of equivalence:

|                                                                         |          |
|-------------------------------------------------------------------------|----------|
| Divalent chromium salt                                                  | 0.1 to 2 |
| Free formic and/or glycolic acid                                        | 0.3 to 1 |
| Alkali formate and/or glycolate, or<br>alkali metal salt of strong acid | 0.3 to 4 |
| Fluoride (when boric acid is present)                                   | 0 to 5   |
| Boric acid                                                              | 0 to 3   |

Within the concentration ranges specified, it should be noted that the more dilute solutions may have lower current efficiencies and/or lower maximum plating ranges. To counteract this disadvantage of low concentrations is the advantage that less chemicals are lost by drag-out of plating solution. At the upper end of the concentration range, we generally do not lose in current efficiency or plating rate or character of deposit. Rather, we are likely to run into solubility limits of the various reacting species in the solution so that precipitation occurs. This does not, of itself, impair plating, but precipitated ingredients obviously are of no utility. Another obstacle at high concentrations is increasing viscosity of the solution, and decreasing conductivity, with correspondingly increased voltage and power consumption. Some of the compositions given in Table I, below, may precipitate crystalline material at room temperature. This does not ordinarily interfere with their useful plating. However, the precipitated material should be left in if one chooses to plate at an elevated temperature, when it will redissolve.

The function of the boric acid in a plating bath of this invention not containing a fluoride is to act directly as a buffer to control pH at the cathode. The presence of boric acid usually broadens the conditions of temperature and current density at which plating is satisfactory. The presence of boric acid increases the current density at which bright chromium can be plated without decreasing the threshold current density at which chromium first deposits. When boric acid is used, and no fluoride is present, the pH should be kept within the range of 1.7 to 3.5. If it is desired to operate a chromium plating bath of this invention at a pH of <2.7, then fluoride should be excluded from the bath because fluoride in the presence of boric acid at pH's lower than 2.7 increasingly reacts to form fluoborate ion,  $\text{BF}_4^-$ , which I find to be useless or even harmful in the system. When boric acid and sodium fluoride are present in the bath together, the pH may be used in the range 2.7 to 4.5.

Under some circumstances it may be desired to plate chromium in accordance with this invention without the presence of fluorine, as noted below. However, when it is desired to attain the broadest working range of current densities and also highest plating rates, then the system containing both boric acid and fluoride is preferred. My experiments indicate that fluoride and boric acid in these plating baths in the pH range of 2.7 to 4.5 react rapidly and almost completely to form the ion  $\text{BF}_3\text{OH}^-$ . In the absence of boric acid, sodium fluoride in this pH range becomes sodium bifluoride by the reaction:



If boric acid is present, however, the following reaction occurs very rapidly:



The  $\text{BF}_3\text{OH}^-$  ion acts as a powerful buffer capable of destroying hydroxyl ions near the cathode by a reaction such as:



When boron and fluorine compounds are placed together in water solution, the useful  $\text{BF}_3\text{OH}^-$  ion is present and

stable in the pH range of 2.7 to 4.5. At higher pH's this becomes unstable relative to bifluoride ion,  $\text{HF}_2^-$ , and free boric acid. At pH's below 2.7 the  $\text{BF}_3\text{OH}^-$  ion becomes unstable relative to the well-known fluoborate ion,  $\text{BF}_4^-$ . These pH limits may not be absolutely sharp, but approximately define the limits of equilibrium stability of the  $\text{BF}_3\text{OH}^-$  ion.

In choosing the amounts of fluorine and boron compounds to be used in preparing my fluorine-containing baths it is desirable to use enough boric acid or equivalent not only to form the  $\text{BF}_3\text{OH}^-$  ion but also to practically saturate the bath with additional boric acid. This procedure tends to stabilize the fluorine as  $\text{BF}_3\text{OH}^-$ . If, on the other hand, an excess of fluoride is used, relative to boric acid, then the excess tends to form a bifluoride such as  $\text{NaHF}_2$  which is only sparingly soluble. There is no sharp dividing line, but in general as the  $\text{BF}_3\text{OH}^-$  ion concentration is raised the working range of current densities of the plating bath becomes desirably broader. A limit on the amount of  $\text{BF}_3\text{OH}^-$  which can practically be used is caused by the fact that bifluoride ions are in equilibrium with  $\text{BF}_3\text{OH}^-$ , and so an excessive concentration of  $\text{BF}_3\text{OH}^-$  may cause precipitation of sodium bifluoride.

The conditions above described are suitable for deposition of bright chromium resembling in good appearance, color, and brilliance the chromium conventionally deposited from hexavalent chromium baths by present commercial processes. This sort of chromium coating imparts not only good appearance, but also surface hardness and a modest amount of additional corrosion protection when used for plating hardware and the like. However, in general, bright chromium deposits of whatever sort have heretofore been usually cracked and always brittle. The literature gives ways of avoiding cracking and improving the over-all corrosion resistance thereby. Even when cracking is avoided, however, all previously-known electrodeposits, including some of those produced in accordance with this invention, are brittle or weak or both. The brittleness and/or weakness is not apparent when chromium is applied as a coating on other metals. However, when the chromium layer is removed, as by dissolving away from it a temporary base metal, the chromium layer is always found to disintegrate into tiny flakes because of inherent brittleness and weakness. I have found within the broad range of conditions of this invention, all of which are suitable for bright decorative plating of metal articles, a narrower range of conditions under which one may deposit chromium which has an exceedingly high tensile strength and under some conditions has a high degree of plastic deformability. These narrowed conditions comprise the following essentials: (1) formic acid with or without formate as the sole carboxylates; (2) a deposition temperature above about 50° C.; (3) substantially complete freedom from sulfur and selenium compounds (less than 10 p.p.m.). When these narrowed conditions are used, it has been noted that plated hardware becomes more resistant to corrosion, after deformation thereof, than when previously-known chromium plating is used. Also, by depositing such chromium films on a temporary metal base, such as brass, it is possible to release sheets of chromium foil when the base metal is dissolved away, as by use of nitric acid. These sheets of foil are in marked contrast to the minute flakes of weak, brittle chromium deposited by other ways, even though the latter may be quite satisfactory for decorative plate. These chromium foils have been found to possess some ductility at thicknesses less than  $50 \times 10^{-6}$  inches. At thicknesses greater than  $50 \times 10^{-6}$  inches, little or no ductility remains, but strength measurements indicate the same high tensile strengths as the thinner films. The tensile strength of chromium electrodeposited by the above-said narrow ranges of conditions has been found to vary between 200,000 to 450,000 lbs. per square inch by actual test on weighted strips. The highest previ-

ously reported tensile strength of chromium is under 114,000 lbs. per square inch. Such thin, ductile and/or high-strength chromium metal films should be of utility where high film strength and exceptional corrosion resistance are desired in metal foils. For example, they may be used advantageously for the metal transfer films of my copending patent application, Serial No. 33,951, filed June 6, 1960. While the ductility and strength of such foils as deposited and released are exceptional for chromium, it is found that these properties can be enhanced by baking the chromium films either before or after release at temperatures from 200 to 350° C. for periods of a few seconds up to one hour. The high tensile strength chromium as produced within the aforesaid narrow ranges of conditions also differs from previously known chromium in its electrical properties. Whereas prior art chromium has an electrical resistivity of  $13 \times 10^{-6}$  ohm cm., this chromium has a resistivity of  $149 \pm 9 \times 10^{-6}$  ohm cm. Moreover, this chromium has a much lower temperature coefficient of resistivity than prior art chromium, i.e.,  $0 \pm 5 \times 10^{-6}$  per degree C. versus about 2,000 to  $3,000 \times 10^{-6}$  per degree C.

With regard to the purity of the chromium deposition bath, I have found that as little as 10 p.p.m. of either sulfur or selenium in the electrolytic plating bath is quite detrimental to the physical strength of the resultant chromium foil. Fortunately, it is relatively easy to eliminate compounds of these elements from my bath by boiling and evaporation. It appears that most sulfur and selenium compounds are reduced by the divalent chromium ion to hydrogen selenide and hydrogen sulfide, which gases are removed with the steam during evaporation. Ordinarily, no special treatment is needed to remove these impurities from my baths, beyond a partial evaporation of the water therein. However, some of the formic acid may also be lost in this evaporation and should be replaced as indicated by analysis of the solution. Even when these impurities were completely removed from a bath containing glycolic acid, a ductile or strong chromium foil did not result even at a deposition temperature of 58° C. Also, by way of comparison, a thoroughly purified solution containing formic acid as the only carboxylic acid did not yield a ductile or strong chromium foil when deposition took place at 25° C.; the same solution yielded both ductile and high-strength chromium foils when the electrodeposition is carried out between 50 and 90° C.

Divalent chromium compounds in solution are oxidized by exposure to air. Hence it is desirable to pad the electrolytic cell with an inert gas such as nitrogen. Another workable process is to keep the bath substantially covered with an inert foam. Such a foam will often form on the bath during use. It may also be desirable to store the previously prepared baths under an inert gas, e.g., nitrogen to minimize air-oxidation of the divalent chromium. A little chromium oxidation does no great harm. The trivalent chromium salts formed by oxidation do not appear to poison or harm the bath. However, if a large proportion of the divalent chromium becomes oxidized to trivalent chromium, the bath stops plating. The amount of chromous ion in the bath must be sufficient that the chromium metal plated out is from the chromous ion rather than the chromic ion.

It may be found advantageous to improve the electric conductivity of the bath by the addition of alkali salts of strong acids (dissociation constant  $> 10^{-2}$ ), such as sodium chloride, bromide or iodide. The foreign anions such as chloride ion may cause some problems at the anode. This may be avoided by placing the anode in a separate compartment with a porous diaphragm to limit mixing of the solution from the anode and cathode regions, or they may be completely avoided by use of a cation permeable membrane. Coatings coated with cation exchange resins are commercially used in preventing transfer of anions while permitting free passage of cations.

7  
8  
Salts of weak acids (dissociation constant  $< 10^{-2}$ ) should not be added except those of essential formic and/or glycolic acids. Such salts of weak acids react with the formic and/or glycolic acids, removing these essential materials. For example, acetic acid (dissociation constant about  $10^{-5}$ ) and acetates are detrimental, increasing so with increasing concentration. It is also to be noted that alkali salts should not be added of those acids whose anions might be reduced at the cathode, such as nitrates.

5 Surf. ca-active agents may be added to the plating baths of this invention. Such agents have several useful purposes. For example, "Petrowet R," a saturated hydrocarbon sodium sulfonate, is advantageously added in 15 amounts of the order of 0.02% to reduce bubble size and improve uniformity of deposition and hence maximum plating speed, i.e., the maximum rate of deposition of bright metal in units of weight per unit area per unit time. Normal octyl alcohol in amounts of the order of 20 0.01% may be added to counteract the excessive foaming tendency of "Petrowet R" and also to reduce any tendency of pitting.

25 Within the range of pH 1.7 to 4.5, the higher the pH the lower the threshold current density (other conditions being held constant) but also the lower the ceiling current density of bright plating. The former is a desirable result but the latter is undesirable. Increasing quantities of un-ionized acids at constant pH has to some extent the same effect as that of a lower pH.

30 The following examples are given to illustrate certain preferred embodiments of this invention.

#### EXAMPLE I

An electrolytic plating bath was made with the following substances in gram-moles per 1,000 grams of solution:

|                                             |     |
|---------------------------------------------|-----|
| Chromium (II) chloride, CrCl <sub>2</sub>   | 0.4 |
| Formic acid, H <sub>2</sub> CO <sub>2</sub> | 0.5 |
| Sodium chloride, NaCl                       | 0.5 |

40 This was electrolyzed at about 55° C. in a cell with a diaphragm, to separate anode and cathode compartments. A platinum anode and a polished brass cathode were used. At a current density of 340 amp./sq. ft. a very bright chromium deposit was obtained at a rate of about 45 65 mic. o-inches per minute and current efficiency of about 20%. When a specimen of the chromium deposit was recovered as foil, by solution of the brass plate in nitric acid, it was found to be 43 microinches in thickness. The foil was exceptionally strong, considering its thinness. 50 When folded double and creased, it did not break in the usual manner of brittle chromium, but retained the creased form.

#### EXAMPLE II

55 One gram-mole of chromium (II) chloride in solution was prepared by reacting at 90-100° C. an excess of commercial pure chromium with two gram-moles of hydrogen chloride in a total volume of 510 ml. of water, the acid being slowly added to avoid excessive reaction speed. The solution was filtered to remove excess 60 chromium metal and evaporated in vacuo to dryness, in order to free it of traces of volatile selenium and sulfur compounds. The chromium (II) chloride was dissolved in water; 0.2 gram-mole of sodium formate and 0.6 gram-mole of formic acid were added; and the solution was made up with water to a weight of 1,000 gm. These operations were conducted under a nitrogen atmosphere. The solution was used for electrodeposition of chromium in the manner set forth in Example I at various temperatures from 25° C to 75° C. and at various 70 current densities from 50 to 420 amp./sq. ft., resulting in very bright chromium deposits, at each temperature over a useful range of current densities. As one instance, electrolysis at 55-60° C. with 280 amp. per sq. ft. yielded an extremely bright plate on a brass substrate, 75 at a rate of 32 microinches/min. and current efficiency

of 11%. The plating was released from the brass substrate, by solution of the latter with a 20% nitric acid solution, as a single sheet of bright foil, with exceptionally high strength.

## EXAMPLE III

0.57 gram-mole of purified chromium (II) chloride was prepared as in Example II. To this was added 1.17 gram-moles sodium formate, 0.57 gram-mole formic acid, 1.33 gram-moles boric acid, 2.90 gram-moles of sodium chloride, and water to a total weight of 1,000 gm. To this solution was added also 0.15% by weight of "Petrowet R," a saturated hydrocarbon sodium sulfonate and 0.1% by weight of normal octyl alcohol, these additions being convenient for improving uniformity of distribution of electrodeposits. This solution, when electrodeposited, yielded very bright electrodeposits over a wide range of temperatures from 7° to 90° C. and current densities from 85 to over 450 amps./sq. ft., the useful range of current densities increasing with temperature.

As exemplary of the effect of deposition temperature on the physical properties of the resultant chromium, there are described below electrodeposits A, B and C. All of these were deposited to the same thickness on brass panels from a bath of the above composition, but respectively at 6° C., 25° C., and 55° C. All the electrodeposited panels were baked at 300° C. for 15 minutes, and then placed in 1:1 nitric acid-water mixture to dissolve the brass. In cases A and B, the chromium was so weak and brittle that it spontaneously disintegrated into small flakes. In case C, however, an exceptionally strong foil resulted having a thickness of about 125 microinches. Direct tensile strength measurements were made on ribbons prepared from this foil. The tensile strengths recorded on different samples of the same were 230,000, >270,000, and 450,000 pounds per square inch. In the case of the lower figures it is believed that accidental edge flaws made during preparation of the test strip were responsible for breakage, and that the highest figure is closer to the true strength of this material.

The following table sets forth the bath ingredients in gram molecular weights of Examples IV to XVII, inclusive. In these examples are also stated the pH value and the maximum rate of bright plating in microinches per minute. The baths of Examples IX and X contain no fluorine. Bath of Example IV contains glycolate ions but no formate ions whereas the bath of Example V contains formate but no glycolate ions, and bath of Example VI contains both formate and glycolate ions. These were all effective for bright plating in the range of 20-300 amperes/sq. ft., the optimum current density, however, tending in all cases to increase with operating temperature.

Table  
MOLAR COMPOSITIONS—DIVALENT PLATING BATHS

| Example No.                      | IV   | V    | VI   | VII  | VIII | IX   | X    | XI   | XII  | XIII | XIV  | XV   | XVI  | XVII |
|----------------------------------|------|------|------|------|------|------|------|------|------|------|------|------|------|------|
| Na <sub>2</sub> CrF <sub>4</sub> | 0.64 | 0.63 | 0.64 | 0.55 |      |      |      |      | 0.26 | 0.55 | 1.10 | 0.55 | 0.26 | 0.13 |
| CrCl <sub>2</sub>                |      |      |      |      | 0.54 | 0.51 | 0.51 | 0.54 |      |      |      |      |      |      |
| NaF                              |      |      |      |      | 2.21 |      |      | 2.21 | 0.61 |      | 0.62 | 2.82 | 3.98 | 4.50 |
| NaHCO <sub>3</sub>               |      |      |      |      | 1.19 | 1.18 |      | 0.41 |      |      |      |      |      |      |
| HCl                              |      |      |      |      |      |      |      |      |      |      |      |      |      |      |
| CH <sub>3</sub> OHCOOH           | 1.92 |      | 0.95 | 0.72 | 0.73 | 0.88 | 0.68 |      | 1.74 | 1.54 | 0.16 | 0.50 | 1.13 | 1.34 |
| HCOOH                            |      | 1.89 | 0.95 | 0.72 | 0.73 | 0.89 | 0.68 | 1.46 |      | 0.19 | 1.98 | 1.43 | 1.14 | 1.01 |
| HCOONa                           |      |      |      |      |      |      |      |      | 0.49 | 1.35 | 1.10 |      | 1.15 | 1.02 |
| H <sub>3</sub> BO <sub>3</sub>   | 1.46 | 1.42 | 1.44 | 3.10 | 3.12 | 1.34 | 1.34 | 3.12 | 2.94 | 1.73 | 3.05 | 3.03 | 3.05 | 3.05 |
| NaCl                             | 3.20 | 3.15 | 3.15 | 2.72 | 1.68 | 2.95 | 2.94 | 1.66 | 3.55 | 3.00 | 3.00 | 3.00 | 2.41 | 2.16 |
| Octyl alcohol                    | .01  | .01  | .01  | .01  | .01  | .01  | .01  | .01  | .01  | .01  | .01  | .01  | .01  | .01  |
| pH                               | 3.18 | 3.30 | 3.08 | 3.32 | 3.32 | 2.48 | 3.11 | 3.49 | 3.87 | 3.89 | 3.79 | 3.79 | 3.75 | 3.87 |
| D <sub>max.</sub> microinch/min. | 25   | 40   | 40   | 35   | 45   | 55   | 5    | 45   |      | 85   | 50   | 45   | 30   | 10   |

## EXAMPLE XVIII

The bath of stoichiometric composition identical to that of Example III was prepared, using instead of CrCl<sub>2</sub>, the compound CrClOH·H<sub>3</sub>BO<sub>3</sub>; amounts of other raw materials were adjusted for this purpose. Electrolytic

tests showed results substantially identical to those of Example III.

## EXAMPLE XIX

5 Electrolytic plating baths identical to that of Example III were prepared with the sole exception that CrCl<sub>2</sub> was replaced respectively with (a) Cr(HCO<sub>2</sub>)<sub>2</sub>·2H<sub>2</sub>O, (b) Cr(CH<sub>2</sub>OH·CO<sub>2</sub>)<sub>2</sub>·H<sub>2</sub>O, (c) CrBr<sub>2</sub>, and (d) CrI<sub>2</sub>. In each case plating results with these modified baths were substantially the same as the results set forth in Example III.

10 The electrolytic plating baths of this invention may contain stabilization agents, wetting agents, oxidation inhibitors or other additive materials commonly used in the plating art, inasmuch as the plating baths herein disclosed have a tendency toward oxidation, both from the air and at the anode as a result of oxygen formation at the anode, it is desirable to maintain the bath closed to the atmosphere or to surround or shield the anode with a layer of paper or other ion-permeable film.

15 The plating baths of this invention and the process of plating therewith has produced bright chromium electrodeposits at current densities of 20 to 450 amps. per sq. ft. The throwing power of the baths is generally greater than that of commercial hexavalent chromium plating baths and current efficiencies of 15 to 40%, based on divalent chromium are obtainable. Comparable current efficiencies of conventional commercial hexavalent chromium plating baths would have to be 45% to 120%, the latter figure being, of course, impossible, whereas such commercial processes usually have efficiencies no greater than 8-12% and at most 20%.

20 Since it is obvious that many changes and modifications can be made in the above-described details without departing from the nature and spirit of the invention, it is to be understood that the invention is not to be limited to said details except as set forth in the appended claims.

25 I claim:

30 1. An aqueous electrolytic plating bath for the plating of bright chromium plate from chromium in the divalent state, said bath having a pH of 1.7 to 4.5 and containing as essential ingredients, per 1,000 g. of bath, 0.1 to 2 gram-moles of a divalent chromium salt, 0.3 to 1 gram-mole of at least one carboxylic acid taken from the group consisting of formic and glycolic acids and 0.3 to 4 gram-moles of at least one alkali metal salt of an acid taken from the group consisting of formic, glycolic and acids having a dissociation constant of at least  $1 \times 10^{-2}$ .

35 2. An aqueous electrolytic plating bath for the plating of bright chromium plate from chromium in the divalent state, said bath having a pH of 1.7 to 4.5 and containing as essential ingredients, per 1,000 g. of bath,

40

45

50

55

55

0.1 to 2 gram-moles of a divalent chromium salt, 0.3 to 1 gram-mole of formic acid and 0.3 to 4 gram-moles of at least one alkali metal salt of an acid taken from the group consisting of formic, glycolic and acids having a dissociation constant of at least  $1 \times 10^{-2}$ .

3. An aqueous electrolytic plating bath for the plating of bright chromium plate from chromium in the divalent state, said bath having a pH of 1.7 to 4.5 and containing as essential ingredients, per 1,000 g. of bath, 0.1 to 2 gram-moles of a divalent chromium salt, 0.3 to 1 gram-mole of at least one carboxylic acid taken from the group consisting of formic and glycolic acids and 0.3 to 4 gram-moles of an alkali metal formate.

4. An aqueous electrolytic plating bath for the plating of bright chromium plate from chromium in the divalent state, said bath having a pH of 1.7 to 4.5 and containing as essential ingredients, per 1,000 g. of bath, 0.1 to 2 gram-moles of a divalent chromium salt, 0.3 to 1 gram-mole of formic acid and 0.3 to 4 gram-moles of an alkali metal formate.

5. An aqueous electrolytic plating bath for the plating of bright chromium plate from chromium in the divalent state, said bath having a pH of 1.7 to 4.5 and containing as essential ingredients, per 1,000 g. of bath, 0.1 to 2 gram-moles of a divalent chromium salt, 0.3 to 1 gram-mole of glycolic acid and 0.3 to 4 gram-moles of an alkali metal glycolate.

6. An aqueous electrolytic plating bath for the plating of bright chromium plate from chromium in the divalent state, said bath having a pH of 1.7 to 4.5 and containing as essential ingredients, per 1,000 g. of bath, 0.1 to 2 gram-moles of a divalent chromium salt, 0.3 to 1 gram-mole of formic acid and 0.3 to 4 gram-moles of an alkali metal salt of an acid having a dissociation constant of at least  $1 \times 10^{-2}$ .

7. An aqueous electrolytic plating bath for the plating of bright chromium plate from chromium in the divalent state, said bath having a pH of 1.7 to 4.5 and containing as essential ingredients, per 1,000 g. of bath, 0.1 to 2 gram-moles of a divalent chromium salt, 0.3 to 1 gram-mole of glycolic acid and 0.3 to 4 gram-moles of an alkali metal salt of an acid having a dissociation constant of at least  $1 \times 10^{-2}$ .

8. An aqueous electrolytic plating bath for the plating of bright chromium plate from chromium in the divalent state having a tensile strength of at least 200,000 lbs. per sq. in., said bath having a pH of 1.7 to 4.5 and containing as essential ingredients, per 1,000 g. of bath, 0.1 to 2 gram-moles of a divalent chromium salt, 0.3 to 1 gram-mole of formic acid as the sole carboxylic acid in the bath and 0.3 to 4 gram-moles of an alkali metal formate as the sole carboxylate in the bath, said bath containing less than 10 p.p.m. of a material taken from the group consisting of sulfur and selenium.

9. Chromium electroplate having a tensile strength exceeding 200,000 lbs. per sq. in. and having an electrical resistivity of  $149 \pm 9 \times 10^{-6}$  ohm cm.

10. The process of electroplating a bright chromium electroplate which comprises passing a direct electric current with a current density of 20 to 450 amps./sq. ft. between an inert anode and a metallic cathode in an electrolytic plating bath having a pH of 1.7 to 4.5 and containing as essential ingredients, per 1,000 g. of bath, 0.1 to 2 gram-moles of a divalent chromium salt, 0.3 to 1 gram-mole of at least one carboxylic acid taken from the group consisting of formic and glycolic acids and 0.3 to 4 gram-moles of at least one alkali metal salt of an acid taken from the group consisting of formic, glycolic and acids having a dissociation constant of at least  $1 \times 10^{-2}$ .

11. The process of electroplating a bright chromium electroplate which comprises passing a direct electric current with a current density of 20 to 450 amps./sq. ft. between an inert anode and a metallic cathode in an electrolytic plating bath having a pH of 1.7 to 4.5 and containing as essential ingredients, per 1,000 g. of bath, 0.1 to 2 gram-moles of a divalent chromium salt, 0.3 to 1 gram-mole of formic acid and 0.3 to 4 gram-moles

of at least one alkali metal salt of an acid taken from the group consisting of formic, glycolic and acids having a dissociation constant of at least  $1 \times 10^{-2}$ .

12. The process of electroplating a bright chromium electroplate which comprises passing a direct electric current with a current density of 20 to 450 amps./sq. ft. between an inert anode and a metallic cathode in an electrolytic plating bath having a pH of 1.7 to 4.5 and containing as essential ingredients, per 1,000 g. of bath, 0.1 to 2 gram-moles of a divalent chromium salt, 0.3 to 1 gram-mole of at least one carboxylic acid taken from the group consisting of formic and glycolic acids and 0.3 to 4 gram-moles of an alkali metal formate.

13. The process of electroplating a bright chromium electroplate which comprises passing a direct electric current with a current density of 20 to 450 amps./sq. ft. between an inert anode and a metallic cathode in an electrolytic plating bath having a pH of 1.7 to 4.5 and containing as essential ingredients, per 1,000 g. of bath, 0.1 to 2 gram-moles of a divalent chromium salt, 0.3 to 1 gram-mole of formic acid and 0.3 to 4 gram-moles of an alkali metal formate.

14. The process of electroplating a bright chromium electroplate which comprises passing a direct electric current with a current density of 20 to 450 amps./sq. ft. between an inert anode and a metallic cathode in an electrolytic plating bath having a pH of 1.7 to 4.5 and containing as essential ingredients, per 1,000 g. of bath, 0.1 to 2 gram-moles of a divalent chromium salt, 0.3 to 1 gram-mole of glycolic acid and 0.3 to 4 gram-moles of an alkali metal glycolate.

15. The process of electroplating a bright chromium electroplate which comprises passing a direct electric current with a current density of 20 to 450 amps./sq. ft. between an inert anode and a metallic cathode in an electrolytic plating bath having a pH of 1.7 to 4.5 and containing as essential ingredients, per 1,000 g. of bath, 0.1 to 2 gram-moles of a divalent chromium salt, 0.3 to 1 gram-mole of formic acid and 0.3 to 4 gram-moles of an alkali metal salt of an acid having a dissociation constant of at least  $1 \times 10^{-2}$ .

16. The process of electroplating a bright chromium electroplate which comprises passing a direct electric current with a current density of 20 to 450 amps./sq. ft. between an inert anode and a metallic cathode in an electrolytic plating bath having a pH of 1.7 to 4.5 and containing as essential ingredients, per 1,000 g. of bath, 0.1 to 2 gram-moles of a divalent chromium salt, 0.3 to 1 gram-mole of glycolic acid and 0.3 to 4 gram-moles of an alkali metal salt of an acid having a dissociation constant of at least  $1 \times 10^{-2}$ .

17. The process of electroplating a bright chromium electroplate which comprises passing a direct electric current with a current density of 20 to 450 amps./sq. ft. between an inert anode and a metallic cathode in an electrolytic plating bath having a pH of 1.7 to 4.5 and containing as essential ingredients, per 1,000 g. of bath, 0.1 to 2 gram-moles of a divalent chromium salt, 0.3 to 1 gram-mole of formic acid as the sole carboxylic acid in the bath and 0.3 to 4 gram-moles of an alkali metal formate as the sole carboxylate in the bath, said bath containing less than 10 p.p.m. of a material taken from the group consisting of sulfur and selenium.

65 References Cited in the file of this patent

UNITED STATES PATENTS

1,922,853 Kissel \_\_\_\_\_ Aug. 15, 1933  
1,975,239 Ungelenk et al. \_\_\_\_\_ Oct. 24, 1934

70 FOREIGN PATENTS

292,094 Great Britain \_\_\_\_\_ Aug. 8, 1929